

## UNITED STATES PATENT OFFICE

2,097,589

## TREATMENT OF TEXTILE MATERIALS

Henry Dreyfus, London, England

No Drawing. Application August 24, 1935, Serial  
No. 37,781. In Great Britain August 30, 1934

8 Claims. (Cl. 91—68)

This invention relates to improvements in the treatment of textile materials, and is more particularly concerned with fixing therein insoluble substances and particularly insoluble metal oxides or compounds. The invention is particularly valuable in the treatment of artificial textile materials, for example those of cellulosic character or those made of cellulose acetate or other organic derivatives of cellulose.

Recently considerable research has been carried out with a view to decreasing or modifying the normal high lustre of artificial silk materials by incorporating therein white opaque compounds, generally insoluble metal oxides or other metal compounds. Proposals to this end have included spinning the artificial silk from solutions containing in suspension the finely divided metal oxides or compounds. Such processes, while yielding artificial silk of dull lustre, necessitate providing stocks of artificial silk both of dull lustre and ordinary bright lustre. Other processes effect a dulling of the lustre of artificial silk after its formation. Such processes involve the successive application of two or more soluble reagents to the materials with resultant precipitation in or on the materials of insoluble metal oxides or compounds. While these processes have the advantage that stocks of artificial silk of normal bright lustre can readily be converted into materials of dull lustre, nevertheless the fastness of the delustering agent upon the material frequently leaves something to be desired. In particular in scouring and in other normal finishing processes, and in domestic washing or other laundering operations, the delustering agent or some of it is liable to be removed with consequent change in the appearance of the artificial silk.

Similarly, for certain purposes it is desirable to load artificial silk not with the object of dulling its lustre but with the object of imparting to it a fuller handle and/or with the object of increasing its safe ironing point or of modifying the dyeing properties. Thus, for instance, artificial silk made of cellulose derivatives may be loaded with tin compounds, for example by treatment with a stannic chloride solution followed by fixation with phosphate and/or silicate solution. It is desirable in order to obtain any substantial loading of the material to apply the tin salt or other solution containing the loading metal radicle under conditions such that the cellulose derivative is in a swollen condition. For example the material may be treated with a swelling agent or a swelling agent may be included in the stannic chloride or similar loading bath, or alternatively the stannic

chloride or similar loading agent may be applied under such conditions of concentration and temperature that it constitutes a swelling agent for the material under treatment. Instead of loading with stannic chloride, phosphate and/or silicate, other insoluble loading agents may be formed in or on the materials, for example phosphates, silicates, borates and the like of the alkaline earth metals, for instance calcium, barium, strontium or of lead or other heavy metals. Some of these metal compounds, particularly the alkaline earth compounds, have the effect of diminishing the lustre of the material in addition to imparting a substantial loading. The silicate, phosphate or like fixing agent, though preferably applied subsequent to the stannic chloride or other metal loading solution, may be applied prior thereto. Where materials containing saponifiable organic esters of cellulose are being treated, the silicate, phosphate or other fixing agent, whether applied prior to or subsequent to the metallic loading solution, may effect a saponification of the cellulose ester. In such loading processes, again the fastness in the material of the loading compound may sometimes with advantage be improved.

In a similar manner insoluble coloured pigments may be formed in or on the material for the purpose of imparting colourations which are faster to light than are the usual dyeings produced with organic dyestuffs. Any lack of fastness to scouring, washing or similar treatments obviously counterbalances the increased fastness to light of the colouring agent.

It is the object of the present invention to improve the fastness to scouring, washing and similar treatments of insoluble substances fixed in or on textile materials. According to the present invention the fastness of such insoluble substances in or on the textile materials is improved by applying to the textiles a film-forming substance insoluble or substantially insoluble in water or the usual scouring liquids. Preferably such film-forming substance is applied in very small amounts so that the properties of the materials as textiles are in no way impaired. Thus, the film-forming materials may be applied to the textiles in very low proportions, and particularly in amounts of under 5% by weight of the textile under treatment. Proportions as low as 3, 2, and 1% or under may be used with advantage and still improve the fastness of the insoluble compounds fixed in or on the textile materials. A further important feature of the present invention consists in applying the film-forming sub-

stances from dilute solutions or dispersions so that little or no sticking of the individual filaments, fibres or yarns of the textiles takes place. For instance with this object in view it is desirable 5 to apply the film-forming substances in solutions or dispersions of a concentration under 5% and preferably as low as 2 or 1% or less.

The difficulty as to the fastness to scouring and similar agencies of insoluble loading, delustring 10 and similar agents arises more particularly with artificial textile materials. Cellulose derivative materials are especially improved by the process of the present invention. As is well known, these materials are relatively impervious to aqueous 15 media and therefore difficulties arise in the loading, delustring and similar treatments of these materials wherein the reagents designed to form in the materials the delustring, loading and similar agents are applied in aqueous media. Usually 20 it is necessary to swell the cellulose derivative during the treatment, and especially during the treatment with a soluble metallic compound. In sufficient penetration of the materials by the aqueous reagents may well be responsible for lack 25 of fastness of the insoluble compound formed on the materials. Probably the smooth character of artificial silk materials also tends to render the loading, delustring or similar agent less fast to scouring, washing and like treatments.

30 The present invention embraces quite broadly the application of any film-forming substance which is insoluble or substantially insoluble in water and in the ordinary scouring and washing baths. A wide variety of film-forming substances 35 is available for the purpose, for example polymerized unsaturated organic compounds generally, for instance polymerized vinyl acetate, polymerized vinyl chloracetate and other polymerized vinyl esters, polyvinylethers, polystyrene and similar polymerized unsaturated hydrocarbons, polymerized unsaturated aliphatic aldehydes, polymerized esters of unsaturated aliphatic acids, for instance, polymerized acrylic ester and polymerized methacrylic ester; various film-forming condensation products, including urea formaldehyde condensation products, phenol aldehyde condensation products and mixed phenol urea aldehyde condensation products, condensation products of polyalcohols with polybasic acids, e. g. the so-called alkyd resins, made, for example, by the condensation of glycerin with phthalic anhydride, and modified alkyd resins, made by reaction between an alkyd resin and an oil or a higher fatty acid. Such polymerization and/or condensation 50 products may be applied in the fully polymerized and/or condensed form, provided they are soluble or dispersible in organic liquids or in aqueous liquids, or they may be applied in a partially polymerized and/or condensed form, with or without 55 subsequent further polymerization or condensation upon the material. If desired the reagents in the unpolymerized or uncondensed form may be applied to the materials and the whole of the polymerization and/or condensation desired effected upon the materials. Generally it is undesirable to employ in such polymerization and/or condensation processes carried out on the materials, temperatures in excess of about 180° C. Preferably temperatures below 150° C. are employed.

70 Other film-forming bodies which are useful for the purpose of the present invention include cellulose and cellulose derivatives, for example nitrocellulose, cellulose acetate, formate, propionate, butyrate and benzoate, methyl-, ethyl- or benzyl-

celluloses or other cellulose esters or cellulose ethers or mixed esters, mixed ethers or mixed ether-esters, for instance oxyethyl cellulose acetate; and solutions of cellulose including viscose and cuprammonium cellulose. The ordinary alkali metal cellulose xanthate solution may be employed or any other soluble or dispersible cellulose xanthate, for example, ammonium cellulose xanthate or a cellulose xanthate of an organic amino base or magnesium cellulose xanthate. Chlorinated rubber is also suitable as a film-forming substance for the purpose of the present invention. Rubber itself is suitable for increasing the fastness of the loading, delustring or other compounds but has the disadvantage that it tends to oxidize in the air, especially in the very thin films in which it is applied according to the present invention. Balata, gutta percha and like bodies have similar properties.

5 As previously indicated, the invention particularly contemplates the application of very small proportions of film-forming substances to the textile materials, and to achieve this low concentrations of the film-forming substances in suitable solvent or dispersion media are especially 10 valuable. The invention more particularly contemplates the application of the film-forming substance to the textile material already loaded with the loading, delustring or other agent.

20 If desired, however, the film-forming substance 30 may, where feasible, be included in one or other of the reagents for forming the loading, delustring or other compound upon the material. Latex, for example, may be included in a neutral or alkaline reagent. Similar remarks apply to 35 the alkali metal cellulose xanthates, ammonium and amine cellulose xanthates and magnesium cellulose xanthate. Thus, for instance, where an insoluble borate, silicate or phosphate is being formed upon the material, such a xanthate 40 or other film-forming substance, stable in the presence of alkali or neutral media, may be dissolved or dispersed in a neutral or alkaline aqueous solution of an alkali metal, silicate, phosphate or borate used for fixing upon the material the 45 loading or delustring metal, for example tin, barium, strontium, calcium and magnesium. The film-forming substance may be included in such a fixing solution, whether the fixing agent be applied before or after the metal salt solution. Further, where feasible a film-forming substance 50 may be dissolved or dispersed in the solution of the salt or other compound of the metal to be fixed in the material, whether the said metal compound be applied before or after the fixing agent.

55 Where the film-forming substance is contained in one of the reagents used for forming the insoluble substance upon the materials, the medium in which it is applied will generally be an aqueous medium. Where it is applied subsequent to the formation on the material of the loading, delustring or other agent, it may be applied either in an aqueous or in an organic medium. Generally the film-forming substances are insoluble in water, so that for application in 60 aqueous media they must be dispersed. However, the film-forming substances may be present in aqueous solution in a soluble form and may be converted upon the material into an insoluble form. Such is the case with viscose and cuprammonium-cellulose and various unpolymerized or uncondensed reagents or partially polymerized and/or condensed substances to be subsequently polymerized or condensed or further polymerized or condensed on the textile material. For in- 70 75

stance, a viscose solution may be applied to a loaded cellulose acetate fabric and may be subsequently steamed or treated with a solution of ammonium acetate, acetic acid, sulphuric acid or other precipitant for the xanthate.

Cellulose acetate and similar cellulose esters, ethers, or ether-esters, the polyvinyl esters, ethers or other compounds, the polymerized acrylic esters and similar polymerized unsaturated esters, and the polymerized aldehydes are most conveniently applied from an organic solvent, for example methyl or ethyl alcohol or other alcohol; acetone, methyl ethyl ketone or other ketone; glycols, glycerine glycol ethers, glycol esters and glycol ether-esters, methyl formate, ethyl formate; methyl acetate, ethyl acetate, butyl acetate and other esters; benzene and its homologues (particularly for dissolving rubber and like substances including polymerized styrene), or mixtures of any of these solvents. Water-miscible solvents may be used in admixture with water, and in fact such aqueous-organic mixtures are very suitable for preventing damage to textiles consisting of cellulose derivatives during the application of the film-forming substance.

Generally the medium in which the film-forming substance is applied to the textile material should have no substantial solvent action upon the textile material. This is particularly important with textile materials made of or containing cellulose derivatives. However, some solvent action of the medium in which the film-forming substance is applied upon the textile material under treatment is advantageous in that it appears to secure a better anchoring of the film-forming substance to the textile material. If desired the film-forming substance may be of the same chemical character as the textile material under treatment. For example a cellulose derivative fabric may be coated with a thin film of cellulose derivative.

It is desirable that the film-forming cellulose derivative shall have different solubility properties from those of the cellulose derivative present in the textile material. If suitable precautions are taken, however, the film-forming substance may be identical or substantially identical with the substance of the textile. For instance a loaded or delustrated cellulose acetate fabric may have a cellulose acetate applied thereto. The film-forming cellulose acetate may be such as will dissolve in a 30-40% aqueous solution of acetone, acetic acid or dioxane at ordinary or high temperatures. Having regard to the low concentrations in which the film-forming substances are preferably applied according to the present invention, this presents no difficulty. A cellulose acetate can readily be prepared which is soluble to the required extent in such an aqueous solvent, even at ordinary temperatures, by arranging the conditions of acetylation, including pre-treatment, acetylation proper and ripening, so as to yield a cellulose acetate of comparatively low viscosity. A suitable cellulose acetate may, for example, be dissolved to a concentration of about 1% in a 20-35% aqueous solution of acetic acid at 70-80° C. and applied in this form to a cellulose acetate fabric. Preferably after the application of the solution the fabric is rapidly cooled. Evaporation of the solvent may be effected at low or relatively low temperatures. Instead of evaporating the solvent, the latter may be so chosen that it is a solvent for the film-forming substance while hot and a non-solvent when cold, so that a hot solution may be applied to the textile and

the film-forming substance precipitated thereon by mere cooling.

The film-forming substance may be applied to the textile materials by any suitable method, for example mechanical impregnation, bath treatments, spraying or the like. Impregnation followed by a squeezing of the fabric so that it retains a predetermined amount of the film-forming solution or dispersion is particularly useful for the purpose of the present invention, since it enables a very uniform application of the film-forming substance in the desired small quantity to be achieved very readily. A loaded or delustrated textile fabric may, for example, be passed through a solution or dispersion of the film-forming substance in a bath or in a padding mangle and the fabric squeezed so as to retain 50, 100 or 150% of its own weight of the solution or dispersion, and the fabric may thereafter be dried or otherwise treated to fix the film-forming substance thereon. A very convenient procedure consists in applying to the fabric a solution of the film-forming substance in a concentration of  $\frac{1}{2}$  to 1 or 2% and subsequently expressing the film-forming solution so that the fabric contains a quantity of 50-100% of its own weight of the solution.

As previously indicated, the process of the invention is of the greatest importance in relation to improving the fastness of loading, delustring or other insoluble substance upon materials made of or containing cellulose acetate or other cellulose derivatives. In this connection reference is made to the delustring or loading processes of U. S. applications S. Nos. 30,944 and 30,945 filed July 11, 1935 and applications S. Nos. 37,779 and 37,780 filed Aug. 24, 1935.

The following examples are given in order to illustrate the invention, but it is to be understood that they do not limit it in any way:

#### Example 1

A fabric of natural silk yarn is steeped in a stannic chloride solution of 40-50° Tw. for half an hour at a temperature of 40-50° C., thoroughly rinsed and then steeped in a solution of disodium phosphate of 4-6° Tw. for half an hour at 40-45° C. The fabric is rinsed, washed in soap solution, rinsed again and then dried.

The dry, loaded fabric is then treated with a 1% solution of cellulose acetate in acetone, passed through nipping rollers to express the solution so that the fabric retains about its own weight of the solution, and dried.

The film of cellulose acetate thus formed on the loaded fabric appreciably reduces the loss in weight occasioned by repeated scouring without changing the appearance of the fabric.

#### Example 2

A fabric of cellulose acetate yarn is steeped for 1 hour at about 20° C. in a loading bath containing about 280 grams of stannic chloride ( $\text{SnCl}_4 \cdot 5\text{H}_2\text{O}$ ) and 243 grams of ammonium thiocyanate per litre. The fabric is removed from the bath, drained well and washed first in two baths of cold water and then in two baths of water at 45° C. until quite free from soluble salts. The fabric is then steeped in a 12% solution of sodium dihydrogen phosphate at 40° C. for half an hour, after which it is rinsed, soaped for 20 minutes at 50° C. in a bath containing 2½ grams per litre of olive oil soap, rinsed and dried.

Polymerized vinyl acetate saponified until it is soluble in 50% aqueous ethyl alcohol is applied

to the dry fabric in the form of a 1½% solution in this solvent, the fabric being passed through nipping rollers to express the solution so that the fabric retains about its own weight of the 5 solution, after which the fabric is dried.

The film of polymerized vinyl acetate thus formed on the fabric appreciably reduces the loss in weight occasioned by repeated scouring without altering the appearance or dyeing properties 10 of the fabric.

*Example 3*

A fabric of cellulose acetate yarn is treated with a fairly concentrated solution of sodium 15 aluminate, centrifuged and then, while still moist, stretched out or hung in a chamber in which it is exposed at 50-70° C. to the moist carbon dioxide. The fabric is then washed until free from sodium carbonate and dried.

20 The fabric loaded with aluminium hydroxide thus obtained is treated with a solution of viscose containing 2% of cellulose for half a minute at 26° C. and squeezed so that it retains about its own weight of solution. The fabric is then 25 placed in a precipitating bath, consisting of a 10% aqueous solution of aluminium acetate, for 2 minutes at 26° C. The fabric is then thoroughly washed and dried.

The fabric thus obtained does not suffer substantial loss in weight even after repeated scouring.

What I claim and desire to secure by Letters Patent is:—

1. In a process for the manufacture of textile 35 materials impregnated with an insoluble metal compound, the step which comprises improving the fastness of said metal compound without substantially impairing the properties of the textile materials by applying to the textile materials 40 impregnated therewith a solution in a volatile organic solvent of a substance which forms a film on the materials which is substantially insoluble in aqueous scouring liquids, the film-forming substance being applied in a quantity less than 5% of the weight of the textile materials treated.

2. In a process for the manufacture of textile 45 materials impregnated with an insoluble metal compound, the step which comprises improving the fastness of said metal compound without substantially impairing the properties of the textile materials by applying to the textile materials impregnated therewith a solution in a volatile organic solvent of a substance which forms a 55 film on the materials which is substantially insoluble in aqueous scouring liquids, the film-forming substance being applied in a quantity equal to ½ to 2% of the weight of the textile materials treated.

60 3. In a process for the manufacture of textile materials impregnated with an insoluble metal compound, the step which comprises improving the fastness of said metal compound without substantially impairing the properties of the textile materials by applying to the textile materials impregnated therewith a solution of less than 5% 65 concentration in a volatile organic solvent of a substance which forms a film on the materials which is substantially insoluble in aqueous scour-

ing liquids, the film-forming substance being applied in a quantity less than 5% of the weight of the textile materials treated.

4. In a process for the manufacture of textile 5 materials impregnated with an insoluble metal compound, the step which comprises improving the fastness of said metal compound without substantially impairing the properties of the textile materials by applying to the textile materials impregnated therewith a solution of ½ to 2% 10 concentration in a volatile organic solvent of a substance which forms a film on the materials which is substantially insoluble in aqueous scouring liquids, the film-forming substance being applied in a quantity equal to ½ to 2% of the 15 weight of the textile materials treated.

5. In a process for the manufacture of textile 20 materials impregnated with an insoluble metal compound, the step which comprises improving the fastness of said metal compound without substantially impairing the properties of the textile materials by applying to the textile materials impregnated therewith a solution of cellulose acetate in a volatile organic solvent so as to form 25 a film of cellulose acetate on the materials which is substantially insoluble in aqueous scouring liquids, the film-forming substance being applied in quantity less than 5% of the weight of the textile materials treated.

6. In a process for the manufacture of textile 30 materials impregnated with an insoluble metal compound, the step which comprises improving the fastness of said metal compound without substantially impairing the properties of the textile materials by applying to the textile materials impregnated therewith a ½ to 2% solution of 35 cellulose acetate in a volatile organic solvent so as to form a film of cellulose acetate on the materials which is substantially insoluble in aqueous scouring liquids, the quantity of cellulose acetate applied being equal to ½ to 2% of the weight 40 of the textile materials treated.

7. In a process for the manufacture of textile 45 materials impregnated with an insoluble metal compound, the step which comprises improving the fastness of said metal compound without substantially impairing the properties of the textile materials by applying to the textile materials impregnated therewith a ½ to 2% solution in 50 a volatile organic solvent of a polymerized unsaturated ester so as to form a film of said ester on the materials which is substantially insoluble in aqueous scouring liquids, the ester being applied in a quantity equal to ½ to 2% of the weight 55 of the materials treated.

8. In a process for the manufacture of textile 60 materials impregnated with an insoluble metal compound, the step which comprises improving the fastness of said metal compound without substantially impairing the properties of the textile materials by applying to the textile materials impregnated therewith a ½ to 2% solution in a volatile organic solvent of vinyl acetate so as to 65 form a film of vinyl acetate on the materials which is substantially insoluble in aqueous scouring liquids, the vinyl acetate being applied in a quantity equal to ½ to 2% of the weight of the materials treated.

HENRY DREYFUS.